

106-18.18

SR

MTR49

XR 1,523,813

18.15

Jan. 20, 1925.

1,523,813

W. G. LINDSAY

CROSS REFERENCE

FIREPROOF FABRIC AND PROCESS OF MAKING SAME

Filed Dec. 14, 1917

Search Room

(1)

Fig. 1.

Fig. 2.



William G. Lindsay Inventor

By his Attorneys

Edwards, Sager & Rower

1523813

OR IN 426/260

## UNITED STATES PATENT OFFICE.

WILLIAM G. LINDSAY, OF NEWARK, NEW JERSEY, ASSIGNOR TO THE CELLULOID COMPANY, A CORPORATION OF NEW JERSEY.

## FIREPROOF FABRIC AND PROCESS OF MAKING SAME.

Application filed December 14, 1917. Serial No. 207,116.

To all whom it may concern:

Be it known that I, WILLIAM G. LINDSAY, a citizen of the United States, residing at Newark, in the county of Essex and State of New Jersey, have invented certain new and useful Improvements in Fireproof Fabrics and Processes of Making Same, of which the following is a specification.

The principal object of my invention is 10 to provide a new and improved coated fireproof fabric for use in various places, and a method of preparing the same. This and other objects will be indicated in connection with the following specification, in which 15 I have disclosed one specific embodiment of my invention and the procedure in accordance therewith.

My improved coated fireproof fabric is especially adapted for use on airplane 20 wings. After the wing frames have been made, the cloth is ordinarily wrapped once around the frame, sleeve-like, and then coated with some varnish-like preparation. It is highly desirable that the fabric be 25 fireproof, but it is difficult to obtain this quality and at the same time get other desirable characteristics, such as waterproofing, strength, flexibility, and a proper shrinkage of the fabric so as to draw it on 30 the frame.

Many attempts have been made to make a non-inflammable coating to be applied to fabrics so that the resulting coated fabric may be fireproof. Many coating substances 35 that have excellent qualities in other respects have not been found available for a fireproof product because they have some degree of inflammability, or because they are not fireproof in themselves to counter- 40 act the normal inflammability of the untreated fabric. Such coating substances as pyroxylin or acetyl cellulose have desirable qualities of water-proofness, shrinking effect, etc., but when applied to a fabric they 45 do not give an effectively fireproof product. By my invention herein disclosed, I have made it possible to employ such substances as those mentioned above, and yet secure fireproofness and the other desirable qualities. 50 Stated in somewhat general terms, according to one aspect of my invention, it involves impregnating the fabric with a

fireproofing substance and then coating it with a coating of reduced or low inflammability, whereby the resultant coated fabric 55 will be effectively fireproof.

The product is shown in the accompanying drawings, in which Figs. 1 and 2 are sections, the latter enlarged, of a fabric coated with the resultant composition. 60

My invention may be practiced in a variety of ways; I will now give one specific example of procedure in accordance therewith. The fabric is first applied to the airplane frame and sewed in place, being 65 drawn to such an ordinary degree of tightness as may be convenient for sewing. Of course, it should be made much tighter than this when ready for service. Next, a water solution of ammonium phosphate is applied 70 with a brush thoroughly saturating the cloth. Then the treated cloth is allowed to dry, leaving it impregnated with the ammonium phosphate.

I prepare a solution of nitrocellulose 75 and tricresylphosphate according to the following formula:

| Parts.             |     |
|--------------------|-----|
| Pyroxylin          | 100 |
| Tricresylphosphate | 50  |
| Acetone            | 300 |
| Methyl alcohol     | 600 |
| Amyl acetate       | 300 |

For the nitrocellulose I use a good soluble 85 variety such as is ordinarily well known to manufacturers of "celluloid." This pyroxylin solution is then applied with a brush and, after it dries, another coat may be applied if so desired and so on to any number of 90 coats. In drying, it shrinks the fabric so as to draw it tight on the frame, increases the tensile strength, the coating unites intimately with the fabric so as to have a unitary character therewith, and leaves a 95 smooth external surface giving a minimum of friction with the air.

In the drawings, the fabric is indicated at A, and the coating composition at B, C.

The dried ammonium phosphate will be in the form of crystals which will adhere to the fibres of the fabric and arrange themselves in irregular manner. The pyroxylin solution will penetrate into the crevices be-

tween the ammonium phosphate crystals and obviously in many places to the fabric itself. At the same time the crystals will be more or less surrounded by and mixed with the pyroxylin thereby forming a more or less intimate mixture between the pyroxylin and the ammonium phosphate, which mixture intimately unites with the fabric to form a unitary structure. If the coating be physi-

- 10 cally separated from the fabric it will carry with it more or less of the ammonium phosphate. The essential functioning of the substances is that they cooperate to provide a fireproofing for the fabric and a waterproofer 15 for the fireproofing and the fabric, the composition also acting to shrink the fabric.

The fabric prepared in this way is effectively fireproof, also waterproof. By "waterproof" I mean not merely that quality which prevents the passage of water through the flexible material but that quality by virtue of which the surface of the material remains intact despite its continued contact with water, this latter quality resulting from the above described treatment. I believe that this action is due to the fact that the crystals are submerged below the surface and are protected by the cellulosic composition. The tricresylphosphate materially reduces the inflammability of the pyroxylin so that the coating alone, that is apart from the fabric, would have a low degree of inflammability. It may be called a coating of low or reduced inflammability. 25 By applying this coating to the fireproofed fabric, such as that treated with the ammonium phosphate, the resultant prepared fabric is thoroughly fireproof.

By suitably varying the process and the ingredients, a variety of so-called artificial leather may be prepared which, unlike many artificial leathers, will be non-inflammable. Various other applications of the process will suggest themselves, such as for fireproofing sails and fabrics in various situations.

The first treatment of the fabric with the ammonium phosphate is for the purpose of fireproofing it and any other suitable fireproofing agent may be employed, such, for example, as ammonium sulphate, or ammonium chloride, or boric acid, or stannic oxide. In the case of airplane wings, the first fireproofing agent can be applied to the fabric either before or after it is put on the frames.

I have employed various proportions of the tricresylphosphate to the nitrocellulose using in different cases all the way from 30 to 100 parts of the former to 100 parts of the latter. In general, the effect of increasing the amount of tricresylphosphate is to decrease the shrinkage of the fabric and to increase the flexibility of the coating.

65 Various suitable solvents may be employed,

such as ethyl alcohol, benzol, ethyl acetate, and ether, in addition to those mentioned in the foregoing formula.

Instead of tricresylphosphate, triphenylphosphate or an ingredient of like effect, 70 may be employed and either of these inflammability reducers may be employed with other coating substances than pyroxylin, if so desired. For example, acetyl cellulose may be used instead of pyroxylin, 75 and in this case less or even none of the tricresylphosphate (or its equivalent) will be required, because acetyl cellulose alone is a substance of low inflammability. Likewise other well known similar substances, 80 known as "dope," containing a volatile solvent which evaporates and leaves a tough flexible waterproof coating, may be employed, with or without a separate inflammability dereaser, according to the nature 85 of the substance.

I claim:

1. The process of making a flexible fireproof coated fabric, which consists in first impregnating the fabric with a solution of a 90 fireproofing substance adapted to give off a fire smothering gas in sufficient quantity to act effectively as a fire retarder, drying the water from said solution, and then coating the impregnated fabric with combustible 95 material containing a fire retarding ingredient, the said coating substance not being a solvent of the said fireproofing substance.

2. The process of making a fireproof 100 coated fabric, which consists in first impregnating the fabric with a water solution of a fireproofing substance adapted to give off water of combination in sufficient quantity to act effectively as a fire retarder, 105 drying the water from said solution, and then coating the impregnated fabric with a combustible composition containing an inflammability reducing substance of essentially different composition from said fireproofing substance.

3. The process of producing a flexible fireproof sheet material which consists in starting with a basic sheet material, making an evenly distributed application of a solution of ammonium phosphate thereto, drying the solvent out of said solution and then coating it with a flexible waterproofing substance having intimately associated therewith an ingredient to render it of low 115 inflammability, said ingredient being essentially different from said fireproofing substance and said coating composition being dissolved in a volatile solvent which is not a solvent of the ammonium phosphate, 120 then evaporating the solvent so as to leave a flexible adherent coat of said composition on the sheet material.

4. A product comprising a fabric coated with a composition containing a fire proof 130

ing substance adapted to give off water of combination in sufficient quantity to act effectively as a fire retarder and a water proofing substance comprising a cellulose ester.

5. A flexible fireproofed coated fabric on a frame consisting of a fabric impregnated with a dried solution of ammonium phosphate and coated with a coating containing 10 a cellulose ester and a fire retarding constituent, the fabric being stretched tightly on the frame by the shrinkage of said coating.

6. The process of making a flexible fire- 15 proof coated fabric which consists in first impregnating the fabric with a solution of fireproofing substance adapted to give off water of combination in sufficient quantity to act effectively as a fire retarder, and 20 then evaporating the solvent from said fire- proofing substance, and then coating it with a flexible coat of low inflammability comprising a cellulose ester, an inflammability reducing substance for said cellulose ester 25 and a solvent, and then evaporating said last named solvent.

7. The process of making a non-inflammable fireproof coated fabric which consists in first impregnating the fabric with 30 a fireproofing substance dissolved in a solvent which is not a solvent of acetylcellulose, evaporating said solvent, and then coating it with a composition containing acetylcellulose and an inflammability re- 35 ducing substance for said acetylcellulose and a solvent which is not a solvent of said fireproofing substance, and then evaporating said last-named solvent.

8. The process of making a fireproof coat- 40 ed fabric which consists in first impregnating the fabric with a solution of fire- proofing salt adapted to give off water of combination in sufficient quantity to act effectively as a fire retarder, drying out the 45 solvent leaving the salt with its water of combination in the fabric, and then applying one or more coats of acetyl cellulose and an inflammability reducer for said acetyl cellulose of essentially different composi- 50 tion from said salt.

9. The process of making a fireproof coated fabric which consists in first impregnating the fabric with ammonium phosphate, and then coating it with a compo- 55 sition containing acetyl cellulose, and an inflammability reducing ingredient for said acetyl cellulose essentially different from said ammonium phosphate.

10. The process of making a flexible fire- 60 proof coated fabric, which consists in first applying to the fabric a fire retarding con- stituent adapted to absorb heat due to the chemical change therein when heated, and then applying a combustible waterproof 65 coating containing an inflammability re-

ducing substance, the said constituents being applied in such relative quantities as to act effectively as to retard fire.

11. The process of making a flexible fire- 70 proof coated fabric which consists in first applying to the fabric a solution of ammonium phosphate, evaporating the solvent, and then applying a coating comprising a mixture of cellulose ester and tricresylphosphate, the ammonium phosphate being present in sufficient quantity to act effectively 75 as a fire retarder.

12. The process of making a waterproof 80 and fireproof coated fabric, which consists in first impregnating the fabric with a solution of a fireproofing substance, adapted to give off water of combination in sufficient quantity to act effectively as a fire retarder, drying the solvent from said substance, stretching the fabric upon a frame, and then coating it with a waterproof coat containing a cellulose ester composition of low inflammability, and drawing said fabric tightly upon a frame by shrinkage of said coating. 85

13. The process of making a fireproof 95 coated fabric shrunken on a frame, which consists in impregnating the fabric with an aqueous solution of fireproofing substance adapted to give off a fire smothering gas containing water in sufficient quantity to act effectively as a fire retarder, and applying it to the frame, evaporating the water from said substance excepting the water of combination, and then coating the fabric 100 with a waterproof coat containing a cellulose ester composition of low inflammability and shrinking it upon the frame by the drying of said coat.

14. A product comprising a cellulose ester 105 and an aromatic phosphate and in close association therewith a fire retarding constituent adapted to give off a fire smothering gas in sufficient quantity to act effectively as a fire retarder. 110

15. A product containing a cellulose ester 115 and an aromatic phosphate and in close association therewith ammonium phosphate in sufficient quantity to act effectively as a fire retarder.

16. A body having on its surface a water- 120 proof material containing a cellulose ester and in close association therewith ammonium phosphate in sufficient quantity to act effectively as a fire retarder.

17. A body having on its surface a ma- 125 terial containing a waterproof combustible constituent and in association therewith a soluble fire retarding constituent adapted to give off a fire smothering gas containing water in sufficient quantity to act effectively as a fire retarder.

18. A product containing in close asso- 130 ciation a cellulose acetate, tricresylphosphate and ammonium phosphate, the two

last named substances being present in sufficient quantity to act effectively as a fire retarder.

19. A product comprising in close association a compound of ammonia, a compound of cellulose and an aromatic phosphoric ester.

20. An article having a surface of tough, plastic material, composed of cellulose acetate plasticized by an aromatic phosphate, said material containing as a fire retarding agent, ammonium phosphate.

WILLIAM G. LINDSAY.